

## UNITED STATES PATENT OFFICE

2,106,888

## SEPARATORY FLOTATION METHOD

Theodore Earle, Pacific Palisades, Calif.

No Drawing. Application June 30, 1936,  
Serial No. 88,148

13 Claims. (Cl. 209—167)

This invention is a continuation in part and a development of my invention as disclosed in my application for Letters Patent of the United States, Serial Number 718,684, and relates to 5 separatory methods for the removal of impurities from material such as sands, sandstones, ores, minerals, and the like, which occur in granular form, and has as an object to provide an improved process or method operable to that 10 end.

A further object of the invention is to provide an improved separatory method particularly adapted for efficient removal of impurities from 15 relatively hard granular material which occurs naturally admixed with a binder having a more or less loose cementing effect on the separate material particles.

A further object of the invention is to provide an improved separatory method particularly efficient in the removal of impurities, discolored particles and particles carrying iron oxide film or 20 coating from natural sands and sandstones.

A further object of the invention is to provide an improved separatory method efficiently operable to float impure, stained, and discolored particles from natural silica sands and sandstones. 25

A further object of the invention is to provide an improved method whereby, through suitable modification thereof, the relative adsorptive powers of various materials may be employed for efficient froth floatative separation of impure, 30 stained and discolored particles from natural silica sands and sandstones.

A further object of the invention is to provide an improved separatory process in the field and for the purpose set forth that is rapid and inexpensive of installation and operation, positive and efficient to the end desired and adaptable to 35 various specific applications.

My invention consists in the various specific 40 steps, and the sequence and combination thereof, set forth hereinafter and pointed out in my claims.

In certain arts, notably that of glass-making, 45 materials occurring in natural granular form, such as silica sands, sandstones, ores, minerals, and the like, are employed, which materials are rarely found free from impurities and are quite commonly admixed with fine particles, clay, soil, 50 and like foreign matter acting as a binder to more or less loosely cement the material particles together, hence it is necessary to submit the natural material to a process effective to separate the particles of the desired material without unduly pulverizing them with consequent 55

production of an undesirably high ratio of fines and to remove the foreign and impure matter from the desired material. In the glass-making art, particularly, it is important that deleterious solid, stained and otherwise discolored particles 5 of the sands employed be removed to prevent discoloration of the ultimate product. Various methods are employed to effect the ends above set forth, but none of the conventional methods at present in use so perfectly attain the desired 10 result in as rapid and economical manner as is possible through use of the improved method herebelow described.

A first and essential step in the improved method is to subject the material under treatment to such action by suitable apparatus as will separate the natural particles of the material from any admixed binder or similar foreign matter and from each other, with a minimum of 15 pulverizing, crushing or splintering of the individual particles, the apparatus to be employed for such purpose being adapted to the character of the specific material to be treated thereby. For example, certain loosely consolidated sands and sandstones may be disintegrated readily by 20 tumbling, or by similar processes of moderate violence; more firmly cemented materials may require violent tumbling or passage through suitable mills arranged to prevent grinding, splintering or crushing of the individual particles, 25 such as chaser mills or mills equipped with rubber covered elements arranged for direct contact with the material. The tightly cemented sandstones and similar materials may require a preliminary crushing to convenient mill size before final disintegration as above set forth. 30 Whatever be the specific method employed, it is essential that the material be thoroughly disintegrated with the least possible destruction of the granular character thereof. "Grinding", as the 35 word is generally understood in the art, does not take place in the apparatus above specified and, being destructive of the individual material particles, is not within the contemplation of the herein described process.

After thorough disintegration of the material, the next step of the improved process involves washing thereof, which may be accomplished through any suitable apparatus in any desired manner to the end of separating the granular 40 material from binder material, soil, clay, trash, soluble material, and other foreign matter admixed therewith. After washing, the cleansed granular material is dewatered, by draining and other suitable methods, to eliminate excess mois- 45 50 55

ture to a degree more specifically set forth hereinbelow, the amount of moisture retained or finally contained by the material having a definite function in the further development of the improved method.

5 Since the technique wherethrough the improved method is made effective is concerned with adsorptive characteristics of the material to be floated and with niceties of water regulation for both of which an adequately specific terminology is not available, certain terms and phrases to be employed in the elaboration of the improved method hereinbelow are herein specifically defined for limitation to the particular meaning readable therein throughout this exposition and the included claims.

*Grain*—"a crystallographic unit as it is seen under the microscope"—Gaudin, pages 131-132.

20 *Particle*—"a small unattached piece of solid—composed of one or more grains. If all the particles in a ground ore are composed of one grain each they are said to be free and the liberation of the minerals by grinding is perfect. If some particles are multigranular, liberation is imperfect. 25 Liberation of the particles of an ore is accomplished by comminution, consisting of crushing and grinding. Ideal comminution consists in breaking the bonds between contiguous dissimilar grains without rupturing the grains."— 30 Gaudin, pages 131-132.

35 The improved process herein described is particularly concerned with and applicable to loose sand, loosely consolidated sands and sandstones, which are "cemented" sands, and hence contemplates comminution of the material to liberation of its constituent particles, one from the other, and avoids, so far as is practicable, such comminution methods as would destroy the identity of the particles or rupture the grains 40 of material.

45 *Adsorptive power*—is used to designate the force with which chemical reagents other than water are attracted to and held on the surfaces of mineral particles; this force varies with the nature of the mineral particle and will vary for a given particle in respect to different reagents.

50 *Adsorptive capacity*—refers to the amount of reagent or thickness of reagent film held to a mineral particle against removal therefrom by a particle of relatively lower adsorptive power.

55 *Affinity*—as herein used means surface attraction and adhesion between a mineral particle and water, only; in other words, the adsorptive power of the mineral as evidenced in respect to water, and not in respect to any other chemical reagent.

60 *Dry*—for purposes of this exposition defines a condition of ore, sand or mineral wherein all water held to the surface of the particles has been removed. This condition can be obtained only through evaporation of the water at temperatures considerably above atmospheric and can be maintained only through maintenance of such temperatures in the ore or mineral, since the material, when at lower temperatures, will adsorb moisture from the air. A dry ore, as here considered, may have free water still within the interior of the particles.

65 *Free water*—refers to the moisture or water content of an ore, sand or mineral other than the water of chemical combination of such material and includes both adsorbed and absorbed water as well as interstitial water. Free water includes all water that can be drained, filtered or evaporated from the ore at temperatures below 70 212 degrees F.

Variable-film water—is herein limited to a designation to the amount of water that can be adsorbed on the exterior surfaces of the various mineral particles and held to these surfaces by the affinity of the particle.

5 *Moist*—defines an ore or sand condition where-in the variable-film water varies from just above the dry condition as a lower limit to an upper limit determined by that total amount of water which can be held to the surfaces of all the particles by affinity. This maximum amount is substantially that which would be adsorbed from the atmosphere of different humidity. The total amount of water used or needed is, of course, determined by the average size of the mineral 10 particles being treated; the finer the size of particles the greater the total surface area and the more water is needed to cover this area to satisfy the affinitive needs of the mass. A sand having a grain size from minus 16 mesh to plus 100 mesh 15 and from which the slimes have been removed will have an upper limit of three percent of water, by weight, to satisfy its affinitive needs while a sand of finer size may need as much as eight percent of water to equally satisfy its affinitive 20 needs. The specific gravity of the material particles may also be a factor. To get the desired flotative effect of variable-film water there must be no interstitial water present, and unless the sand is in the proper condition to start with, 25 evaporation must be employed to eliminate any excess water, since under no conditions can the small amount required by the improved process be obtained by natural drainage alone, or water must be added to bring the material to the desired 30 moist condition. If natural drainage is used as a step in the dewatering of the material, it must be supplemented by evaporation or other similar means. A sand in the moist condition may have some free water absorbed within the interior of 35 the particles, but this water has no harmful effect on the actual flotation of the desired particles. The improved method, as described, deals entirely with the materials in the moist condition. Moisture, as herein used, has the same limitations 40 of meaning as are above employed in respect to 45 moist.

50 *Wet*—refers to that condition of a material where there is sufficient free water to give an excess over that needed to satisfy the affinitive 55 needs of the particles of sand or ore. A sand which has been allowed to drain naturally for a long time but which has not undergone any other treatment for the removal of excess water, is in the wet condition.

55 Continuing the description of the improved method, the moist, cleansed particles of the material under treatment are next mixed with the proper reagent before going to the froth flotation cell. Experiment has definitely established 60 that, by employing a suitable organic reagent, and more especially one of the fatty acid group, both coarse and fine silica particles and similar non-metallic, granular materials may be completely floated. This complete flotation is obtainable when the moist material particles are mixed with the reagent, as above described, since the adsorptive power of such non-metallic particles for fatty acids is relatively low and is not sufficient to effect a flotatively effective concentration 65 of the reagent on and about such particles when carrying a thick water film, a very slight excess of water increases this water film to such an extent that it acts as an inhibitor and prevents the adsorption of the reagent by the pure silica par-

5 ticles. Further, it has been definitely established that certain impure, discolored, and stained particles remaining after washing of the material have adsorptive powers for the fatty acids and their derivatives which are higher than those characteristic of the clean-surfaced, pure silica particles. This higher adsorptive characteristic doubtless results from the metallic nature of the substance or compound contained in or 10 as a film covering on these certain grains. The difference in adsorptive power will vary according to the degree of impurity, stain or discoloration presented in a given instance. This difference in adsorptive powers for certain reagents 15 of the pure and impure particles having been established, eliminative selection of the impure particles can readily be had through a conventional froth flotation cell in the presence of an organic reagent, such as oleic acid and the like, 20 by adjusting the free water content of the washed material and admixture thereof with the reagent so that there will be a sufficient amount of water present to prevent effectively flotation combination between the reagent and the particles characterized by lower adsorptive powers for the reagent used; only those particles having higher 25 adsorptive powers being thus floatable.

30 The amount of free water necessary to effect the selective separation just above described will vary with the specific material under treatment and with the degree of separation to be obtained. In the case of certain silica sands it may be desirable, after disintegration and washing of the material, to dry the washed material, then add 35 the proper amount of water and thoroughly mix it with the material, or allow the sand to take up water from the air, the reagent then being added to and thoroughly mixed with the water-regulated material prior to agitation thereof in 40 the flotation cell. A further step is frequently of advantage with sands and consists in leaving the mixed water-regulated material and reagent in intimate contact for a predetermined length of time prior to introduction thereof into the 45 flotation cell, thus permitting the reagent to thoroughly establish its combination with the particles of higher adsorptive powers prior to dilution of the reagent in the flotation medium.

50 With a relatively higher moisture content in the material, all of the particles have their affinities for water satisfied so that only certain of the more impure particles will float readily in the cell, a relatively lower moisture content acting to progressively float more of the stained and 55 discolored particles as said moisture content is reduced to the minimum, beyond which the particles having the lower adsorptive powers will be 60 filmed with the reagent and float. Where the moisture content of the mixture is below eight percent by weight of the material, the reagent is mixed with the material prior to introduction of either to the flotation cell, and the resulting mixture is thoroughly agitated to uniformly 65 spread the reagent therethrough.

65 Where sand carries impure grains which are easily floated, the material may be deslimed, partially dewatered, as is standard flotation practice, and put directly into the flotation cell where the reagents are added, less than one percent of 70 reagent by weight of the material being required for satisfactory results with this form of the method. This treatment will not remove the minerals of lower adsorptive powers nor iron stained grains. The tailings are then removed 75 from the cell, the moisture content thereof regu-

lated and, after mixing with the proper reagents, the mixture is again put through the flotation cell for further purification.

Once the mixture of material and reagent has been put in the flotation cell, the concentrate 5 should be removed as soon as possible. If the material is allowed to "condition" in the cell for any considerable length of time the film of reagent surrounding the particles in the froth may be washed off with a consequent loss of concentrate. 10 This is especially true where the pure silica particles are being floated, since the silica grains, having a higher affinity for water than adsorptive power for oleic acid or similar reagents, will have the film of reagent removed and 15 replaced by water film, and they will then sink out of the froth. One advantage of the improved method is derived from the unstable froth carrying the concentrate, since the very rapid formation of the concentrate-bearing froth and 20 the necessity for its rapid removal increases the capacity of the cell unit materially.

Where the sand particles are coarse, from minus sixteen to plus eighty mesh, it has been determined that as little as one tenth of one 25 percent (0.1%) of variable-film water, by weight of material, may prevent the flotation of the cleaned silica particles. The finer the sand particles, the more water may be needed to prevent their flotation, as the surface area to be water- 30 film is proportionately increased. The free water content of the material before being mixed with the reagent may vary within narrow limits according to the fineness of the separation desired and the practical considerations involved. 35 For most efficient results the sand should carry less than eight percent of free water by weight before being mixed with the reagent.

Different sands require different treatments 40 depending on the type of impurities to be removed. If a silica sand contains impurities such as biotite mica, magnetite, specular hematite, et cetera, only, these can be floated away from the pure silica particles by keeping sufficient water film around all the sand particles to prevent the adsorption of the reagent by the silica 45 particles but not enough to prevent such action by the impure particles. With most sands of this class not less than one half of one percent (0.50%) moisture must be present before mixing with the reagent, since, with less than this amount of water, there is danger of floating some of the pure silica particles. If the sand 50 particles are fine it may be necessary to have three to eight percent of moisture present to prevent the flotation of the pure silica particles and give a clean concentrate of the impure particles. The best amount of moisture to be used for each sand can readily be determined by simple test. Other sands do not contain the above minerals 55 but do contain certain dark colored and other particles that can be separated from the silica particles by keeping the moisture content below one half of one percent (0.50%) before mixing with the reagent. In this case, best results 60 are usually obtained if the water film on the particles is kept at a minimum. Such sands, when mixed with a fatty acid, such as oleic acid, in amounts of between one tenth pound and five pounds per ton, will have the pure silica particles, only, covered by the reagent and can be 65 separated in a flotation cell. The best amount of reagent to be used for the sand in question must be determined by test. Care must be used 70 not to employ too much reagent, as excess re- 75

agent washes off in the cell and prevents frothing.

Where sands contain a mix of the two kinds of impurities mentioned above, the procedure would be; first, after desliming, the free water content is regulated to that amount which will permit adsorption of the reagent by the mica, garnet, et cetera, but prevent such adsorption by the other grains, the water-regulated material then mixed with the reagent, allowed to stand for time-conditioning, if necessary, and then introduced into a flotation cell for froth floatative separation of these impure particles; second, the tails from the first operations are then dried and again water-regulated to the proper moist condition, mixed with more reagent, time-conditioned, if necessary, while still in the moist condition, and again introduced into the flotation cell for separation of the pure silica particles as a froth concentrate from the impure particles remaining as tails in the cell.

The specific reagent employed may be one of the fatty-acid or soap group or a derivative thereof, and since certain of such reagents are not liquid at normal temperatures, it may be desirable to mix the reagent and material at a temperature above normal, though said temperature should be held below that point where too rapid evaporation of the water in the mixture would result. Oleic acid functions well in the improved method at normal room temperatures.

It is usually desirable and on occasion necessary to add a frother, such as pine oil, terpineol, or the like, to the mixture under treatment, during or prior to agitation thereof in the flotation cell, the frother aiding in the froth flotation effect produced by such cell, as is well known practice.

Certain tests, employing the new method, have resulted as follows:

A natural sand screened to minus thirty plus one hundred mesh was found to carry fourteen one-hundredths (0.14%) of  $Fe_2O_3$ . This sand was deslimed, dewatered to a six percent free water content and treated according to the improved method with three-fourths of a pound of oleic acid to each ton of sand. Impure grains amounting to one-half of one percent (0.50%) of the treated sand weight were floated and thus selectively eliminated, the sand after treatment testing forty-two one-thousandths (0.042%)  $Fe_2O_3$ . By no other method were results obtained which could compare favorably with those above set forth in respect to either lower iron content or cheapness of operation.

A glass sand from Southern California containing solid particles of garnet, magnetite, specular hematite, et cetera, pure silica particles, and particles of lower adsorptive power, such as feldspar, mica, et cetera, was thoroughly disintegrated and cleaned of its slimes by treating the material while wet in a rubber-lined rod mill wherein rubber-covered steel rods were employed to separate the particles and rub them free from slime. The slimes were then discarded, the sand dried and screened to minus twenty plus eighty mesh. This material then showed 6.6%  $Al_2O_3$  and .085%  $Fe_2O_3$ .

A. 500 grams of the above sand was thoroughly mixed with 25 cc. of water and then thoroughly mixed with three drops (.3 lb. per ton) of oleic acid. This mixture was then put through a 1000 gram flotation cell with 2 drops (.2 lb. per ton) of pine oil added as a frother. The froth concentrate resulting from the above

weighed 7 grams and consisted of the solid particles, such as garnet, et cetera.

B. The tails from the foregoing paragraph were dried and then water-regulated to that amount of free water adsorbable from the atmosphere and 200 grams thereof was mixed with 4 drops (1 lb. per ton) of oleic acid, which mixture was then put through the same flotation cell with 2 drops of pine oil. The concentrate resulting from this treatment weighed 170 grams and contained 5.8%  $Al_2O_3$  and .038%  $Fe_2O_3$ , while the tails weighed 30 grams and contained 9%  $Al_2O_3$ .

C. 200 grams of the same material was mixed exactly as in "B" and allowed to stand 24 hours before it was put through the same flotation cell with the same quantity of pine oil. This test produced a concentrate weighing 199 grams and tails weighing 0.73 gram containing mica, et cetera.

The foregoing tests show that:

A. Proper treatment of the clean sand regulated, in this instance, to 5% of moisture permits the flotation of certain grains but prevents the flotation of the silica and lower adsorptive powered grains, and,

B. With the material regulated to that amount of moisture adsorbable from the atmosphere, or less the mix of material and reagent, when immediately floated, permitted the separation of the silica from the feldspar and other impure grains. The feldspar, in this case, has a lower adsorptive power for the oleic acid than has the silica and, even though there is an excess of reagent present beyond the needs of silica, the feldspar does not adsorb at once and hence a separation of the two kinds of grains can be made in the flotation cell.

C. Through time-conditioning of the mix, while in this moist condition, in this instance for twenty-four hours, the weaker feldspar particles are given opportunity to adsorb the oleic acid and are then floated off with the pure silica particles. The particles still remaining as tails would require for their flotation a greater amount of reagent than was supplied for the test.

D. Through regulation of the amount of moisture in the mix, regulation of the amount and kind of reagent, and regulation of the time of contact between reagent and material while in the moist condition, it is possible to floatatively effect separations of the various minerals as given. This can be done only through application of the above described method.

E. By elimination of the fines and the use of small amounts of material in the tests, the worst possible flotation conditions were provided. The fact that the various separations were made under such conditions clearly evidences the novelty of the method. In no other way can such coarse silica grains be floated.

Since variations and modifications in the specific nature and sequence of the steps comprised in the improved method may be had, and may in fact be highly expedient in applying the method to specific materials, all without departing from the spirit of the invention, I wish to be understood as being limited solely by the scope of the appended claims rather than by any details of the foregoing exposition.

I claim as my invention—

1. The method of purifying naturally granular material which comprises disintegration of said material to its constituent elements without crushing or splintering of the particles, washing

of said material and discard of slimes therefrom, dewatering of said material to a water content less than will satisfy the affinitive capacities of all of the separated particles and to that minimum 5 essential for selective flotatively effective limitation of the adsorptive powers of the particles relative to flotation reagents, agitation of said water-regulated material with a fatty acid and agitation of said mixture in a froth flotation cell for 10 separation and removal of impure particles 15 through said cell:

2. The method of purifying naturally granular material which comprises non-destructive disintegration of said material to its constituent particles, washing of the disintegrated material and 15 discard of slimes therefrom, regulation of the water content of the material to an amount less than will satisfy the affinitive capacities of all of the separated particles of the material, agitation 20 of said water-regulated material with one of the soapy reagents, and separation in a froth flotation cell of those material particles having the higher adsorptive powers from the particles of 25 lower adsorptive powers.

25 3. The method of purifying sands which comprises non-destructive disintegration of the sand to its constituent particles, washing of the disintegrated sand and discard of slimes therefrom, drying of the sand, addition to the dried sand of 30 that minimum proportion of water below an upper limit less than will satisfy the affinitive capacities of all of the separated particles and which will sufficiently limit the effective adsorptive powers of the material to prevent flotatively effective adsorptive affiliation between a fatty acid and the 35 pure silica grains, admixture of said water-regulated sand with a fatty acid, and subsequent agitation of the resultant mixture in a froth flotation cell for separatory flotation of the impure particles.

40 4. The method of purifying sands which comprises non-destructive disintegration of the sand to its constituent particles, washing of the disintegrated sand and discard of slimes therefrom, addition to the dried sand of that minimum proportion of water below an upper limit less than will satisfy the affinitive capacities of all of the separated particles and which will sufficiently limit the effective adsorptive powers of the material to prevent flotatively effective adsorptive affiliation between a fatty acid and the pure silica 45 grains, admixture of said water-regulated sand with a fatty acid, prolongation of contact between said reagent and water-regulated sand a determined length of time to the end of selective concentration of said reagent on and about the impure particles characterized by higher adsorptive powers, and subsequent agitation of the resultant mixture in a froth flotation cell for separatory flotation of said impure particles.

45 5. The method of purifying naturally granular material which comprises blunging of the material for disintegration thereof without crushing or splintering of the natural material particles, 50 washing of the blunged material for discard of slimes therefrom, drying of the granular material, thorough mixing of the dried material with a minimum proportion of water below an upper limit less than will satisfy the affinitive capacities of all of the separated particles and which will sufficiently limit the effective adsorptive powers of the material to prevent flotatively effective adsorptive affiliation between a fatty acid and the material particles of lower adsorptive powers, 55 thorough admixture of the water-regulated ma-

terial with a fatty acid to the end of selective concentration of said reagent on and about the material particles characterized by higher adsorptive powers, and subsequent agitation of the resultant mixture in a froth flotation cell for separatory 5 flotation of the impure particles.

6. The method of purifying naturally granular material which comprises blunging of the material for disintegration thereof without crushing or splintering of the material particles, washing of the blunged material for discard of slimes therefrom, drying of the granular material, thorough mixing of the dried material with a minimum proportion of water below an upper limit less than will satisfy the affinitive capacities of all of the separated particles and which will sufficiently limit the effective adsorptive powers of the material to prevent flotatively effective adsorptive affiliation between a fatty acid and the material particles of lower adsorptive powers, thorough ad- 10 mixture of the water-regulated material with a fatty acid, prolongation of contact between said reagent and water-regulated material a determined length of time to the end of selective concentration of said reagent on and about the material particles characterized by higher adsorptive powers, and agitation of the resultant mixture in a froth flotation cell for separatory flotation of the impure particles.

25 7. The method of purifying glass sands and naturally granular ores which comprises disintegration of the material without grinding and consequent crushing or splintering of the material particles, washing of the material and elimination of the slimes therefrom, dewatering of the granular material to a water content less than will satisfy the affinitive capacities of all of the separated particles, agitation of the dewatered material with less than one percent, by weight, of a fatty acid, and subsequent separation of the pure and impure material particles in a froth flotation cell.

30 8. The method of purifying naturally granular ores which comprises disintegration of the material without grinding and consequent crushing or splintering of the material particles, washing of the material and elimination of the slimes therefrom, dewatering of the granular material to a water content less than will satisfy the affinitive capacities of all of the separated particles, agitation of the dewatered material with less than one percent, by weight, of a soap, and subsequent separation of the pure and impure material particles in a froth flotation cell.

35 9. The method of purifying naturally granular ores which comprises disintegration of the material without grinding and consequent crushing or splintering of the material particles, washing of the material and elimination of the slimes therefrom, drying of the granular material, addition to the dried material of water in an amount less than will satisfy the affinitive capacities of all of the separated particles, admixture of the water-regulated material with less than one percent, by weight, of a fatty acid, and subsequent 40 agitation of the resultant moist mixture in a froth flotation cell for separation of the pure and impure material particles.

45 10. The method of purifying sands which comprises non-destructive disintegration of the sand to its constituent particles, washing of the disintegrated sand, regulation of the water content of the sand to substantially that minimum adsorbable by the sand from the atmosphere for 50 selective flotatively effective limitation of the 55

adsorptive power of the sand particles relative to flotation reagents, agitation of said water-regulated sand with a fatty acid and subsequent agitation of said mixture in a froth flotation cell for separation and removal of impure particles through said cell.

11. The method of purifying sands which comprises non-destructive disintegration of the sand to its constituent particles, washing of the disintegrated sand, regulation of the water content of the sand to substantially that minimum adsorbable by the sand from the atmosphere for selective flotation effective limitation of the adsorptive power of the sand particles relative to flotation reagents, agitation of said water-regulated sand with a soapy reagent and subsequent agitation of said mixture in a froth flotation cell for separation and removal of impure particles through said cell.

12. The method of purifying sands which comprises non-destructive disintegration of the sand to its constituent particles, washing of the disintegrated sand, regulation of the free water content of the sand to that minimum less than will satisfy the affinitive capacities of the separated particles effective for flotation inhibition of the silica particles in the presence of a fatty acid, agitation of said water-regulated sand with a fatty acid, agitation of the resultant mixture in a froth flotation cell for separation of impur-

ities as a concentrate from said sand, water-regulation of the tailings from said flotation cell to that minimum free water content effective to permit flotation of the silica particles in the presence of a fatty acid, agitation of said finally water-regulated sand with a fatty acid, and agitation of the resultant mixture in a froth flotation cell for recovery of pure silica particles as a froth concentrate.

13. The method of purifying sands which comprises non-destructive disintegration of the sand to its constituent particles, washing of the disintegrated sand, regulation of the free water content of the sand to that minimum less than will satisfy the affinitive capacities of the separated particles effective for flotation inhibition of the silica particles in the presence of a soapy reagent, agitation of said water-regulated sand with a soapy reagent, agitation of the resultant mixture in a froth flotation cell for separation of impurities as a concentrate from said sand, water-regulation of the tailings from said flotation cell to that minimum free water content effective to permit flotation of the silica particles in the presence of a soapy reagent, agitation of said finally water-regulated sand with a soapy reagent, and agitation of the resultant mixture in a froth flotation cell for recovery of pure silica particles as a froth concentrate.

THEODORE EARLE. 30